

## UNITED STATES PATENT OFFICE

2,107,343

## PROCESS OF TREATING PAPER

5 Chester D. Rockwood and Kenneth L. Osmun,  
 Cincinnati, Ohio, assignors to The Union Sell-  
 ing Company, Cincinnati, Ohio, a corporation  
 of Ohio

No Drawing. Application April 14, 1936,  
 Serial No. 74,341

5 Claims. (Cl. 8—20)

Our invention is concerned with a process of 5 treating paper in order to produce certain desirable results, and is a continuation in part of our copending application Serial No. 31,362, filed July 15, 1935. In that application we disclosed a process of treating paper and the like, in order to obtain certain advantageous qualities, and also a packing material made from such treated material. In this application we have carried the 10 process farther, and have produced a material which has other very advantageous qualities, which will be described hereinafter.

Generally speaking, the treatment of paper with zinc chloride ( $ZnCl_2$ ) is well known in the art. 15 The product of such treatment is a permanently brittle sheet, and this process is therefore used where it is desired to manufacture stiff board, for articles which do not require bending or folding.

20 Genuine vegetable parchment is produced by treating stock with sulphuric acid ( $H_2SO_4$ , specific gravity about 1.69). The sulphuric acid reacts with the starch in paper to form a surface coating of amyloid ( $C_6H_{10}O_5$ ), which is waterproof. A type of parchment is also said to have been produced by the use of weak acids, organic 25 and inorganic, and acid salts, with or without formaldehyde (HCHO). Such a teaching is made in a patent to Fues, No. 1,082,757, dated July 23, 1912. It has been shown, however, ("Separation of cellulose particles in membranes of cotton fibres by treatment with HCl" by Wanda K. Farr and Sophia H. Eckenson—reprint from "Contributions from Boyce Thompson Institute", vol. 6, 30 pp. 309—313, 1934) that weak acids will completely dissolve the cementing materials between the cellulose particles, making the sheet necessarily brittle due to the crystalline structure of the remaining cellulose.

40 Thus it has been shown that weak acids with or without formaldehyde, and zinc chloride alone, do not produce a satisfactory sheet. With the above facts in mind, it is an object of our invention to produce a sheet which will have improved qualities as to stretchability, tensile strength (Elmendorf test), surface tension (Mullen test), tearing strength (Schopper test), waterproofness, toughness, pliability, softness, "feel", leatheriness, and packing qualities. These qualities generally are included in the term "parchment-like effect" as used in the claims.

45 Further objects include the provision of a sheet which will not disintegrate upon prolonged saturation in water, and which will be impervious 50 to strong acids, alkalies, salts, soap solution and

the like, with the exception of concentrated sulphuric acid and sodium hydroxide.

These and other objects of our invention which will be pointed out hereinafter or which will be apparent to one skilled in the art upon reading 5 these specifications, we accomplish by that process which we shall now describe in an exemplary manner.

Briefly, in the practice of our invention, we 10 treat paper, cotton or cellulose fibres with a solution comprising equal parts by weight of zinc chloride (commercial or technical grade), and formaldehyde (commercial forty per cent grade); water may be added if it is desired to dilute the mixture, but the resultant sheet will be less satisfactory, up to a point beyond which the addition of water will prevent the production of our 15 sheet entirely. These materials are mixed until the solids are completely dissolved. Since the solution is an exothermic reaction, the mix must 20 be cooled, and since dirt particles are usually present in the zinc chloride, it must be strained.

The fibre to be treated is conducted through 25 a bath of this solution in such a way as to completely saturate it. Excess moisture is evaporated off by dry heat at a temperature of 100° C. It is to be understood that variation in heat, time of 30 immersion, strength of the solution and the like, will produce variations in the qualities of the finished stock, although in any event the above 35 outlined qualities will be exhibited in varying degrees. Furthermore, the formula recommended by us may be unsuitable for certain types of fibres, and necessary changes must be made accordingly.

The dried sheet, which at this stage of the process 40 should contain at least ten percent moisture, is then conducted through hot calender rolls, whereby the fibre, while it is in a soft gelatinous condition, is ironed or mashed together into a more or less homogeneous film. This condition is readily apparent from the condition of the sheet.

The sheet will now be quite hard, and tending 45 toward brittleness, but on standing, it will take up moisture and become soft and pliable, assuming the characteristics of cloth, leather and parchment. The tensile strength at this point is markedly increased, an effect which we attribute to the action of the zinc chloride which 50 sets up a hydrolysis within the fibres and expands them to several diameters, thereby increasing the matting effect within the sheet and the friction of one fibre over another. The heavy calendering which it has undergone also has consid- 55

erable effect on the strength. This standing of the sheet in air, we term "air conditioning" the sheet. This air conditioning is for the purpose of softening the sheet. It is accomplished by the hygroscopic action of the zinc chloride in the sheet. If this air conditioning step is eliminated, substantially the same result is achieved when the sheet is washed.

The air conditioned sheet is now conducted 10 through a tank of water and scrubbed. By this treatment the zinc chloride and formaldehyde are entirely removed, and the sheet is then normally dried and calendered to the desired finish. The finished sheet we have found to be tough, 15 strong, flexible, leathery, and inert to disintegration in water. It is inclined to stiffness, but it is not brittle and may be folded indefinitely without fracture. When immersed in water, the sheet retains its toughness and tensile strength, 20 but loses its stiffness and becomes more flexible and pliable.

Our sheet must not be compared with any form of parchmentized sheet now known. In parchment paper only the surface is changed, 25 due to the speed at which the operation occurs. This speed is necessary to prevent complete destruction of the sheet. In regard to true vegetable parchment, it must be realized that these papers are seldom made in more than 40# basis 30 weights. The caliper is proportionately less, due to its treatment and calendering. Because of this, it seems as though the sheet were parchmentized throughout, which however is not the case; a microscopic test will show otherwise. A 35 sheet treated in accordance with our process, on the other hand, being of a heavier caliper, readily shows on tearing, that the treatment is complete. Our treatment completely saturates all fibres and the reaction is carried to the endpoint, and of 40 course the treatment is complete. Parchmentizing produces qualities such as water, moisture, and to a certain extent, greaseproofness. We do not claim these qualities with the exception of waterproofness, and perhaps greaseproofness, 45 but we do claim qualities which parchment does not have; viz, leatheriness, toughness, non-disintegration in water, tensile strength and an appearance and "feel" hitherto unknown in the paper converting industry. It is an accepted fact 50 that some parchment is difficult to disintegrate in water, but it more or less retains its stiff, almost brittle characteristic, even when wet, and is not comparable to our sheet in softness. By our treatment, the paper is given a soft, chamois-like 55 quality when wet, but retains its original strength and toughness for many months in this condition.

While we realize that we are not required by the patent laws to state the theory behind our 60 invention, we feel it may be helpful to set forth what we believe to be the reasons for our novel results. The cementing material in the fibres is composed largely of a mixture of pectic materials. Undoubtedly there are also traces of many other 65 substances within the living cytoplasm of the cells which compose the fibres; among these may be hemicellulose, lignin, galactose, albumin, haemoglobin, chlorophyll and the like. This cementing material, instead of being dissolved, undergoes

a complete chemical substitution. Formaldehyde has an acid reaction, and although it does not combine entirely with the alkaline zinc chloride, it does render the mixture active. The pectin, which is a constituent of the cell wall, and 5 closely related to the vegetable gums, is thereby converted to pectic acid by hydrolysis due to the presence of pectase (a diastase) in the cell wall which is energized by the formaldehyde.

Pectic acid is a tough horny mass when dry, 10 but readily becomes soft and gelatinous, although retaining its strength, when wet. Therefore it is our theory that this tough mass combines the cellulose particles into a tougher, tighter, less destructible sheet when dry and simultaneously 15 a soft, pliable sheet when wet, which, however, retains its strength. The untreated sheet, containing pectin, is obviously much weaker.

Therefore, we believe that the peculiar and unique condition of the finished sheet which we 20 desire, is the direct result of the action of the formaldehyde-zinc chloride solution on the pectin present in the cell, changing it to pectic acid and producing the sheet which we have described.

The term "commercial formaldehyde" as used 25 by us in the specification and claims, refers to the formaldehyde available on the market today, which usually comprises in the vicinity of forty per cent by weight of formaldehyde dissolved in water.

Having now described our invention, what we 30 claim as new and desire to secure by Letters Patent, is:—

1. A method of treating paper stock to produce a parchment-like effect which comprises conducting said stock through a bath of a solution of commercial grade zinc chloride in commercial forty per cent grade formaldehyde, said solution being prepared by dissolving the zinc chloride in the formaldehyde solution. 40

2. A method of treating paper stock to produce a parchment-like effect which comprises conducting said stock through a bath of a solution of commercial grade zinc chloride in commercial forty per cent grade formaldehyde, said solution 45 being prepared by dissolving the zinc chloride in the formaldehyde solution, and washing it to remove all traces of said zinc chloride and formaldehyde.

3. A method of treating paper stock to produce 50 a parchment-like effect which comprises conducting said stock through a bath of a solution of one part by weight of zinc chloride in one part by weight of a solution of commercial formaldehyde, said solution being prepared by dissolving 55 the zinc chloride in the formaldehyde solution.

4. A method of treating paper stock to produce a parchment-like effect which comprises conducting said stock through a solution prepared by dissolving commercial zinc chloride in the water 60 of solution of commercial grade formaldehyde.

5. A method of treating paper stock to produce a parchment-like effect, which comprises conducting said stock through a bath of zinc chloride dissolved in the water of solution of commercial 65 formaldehyde.

CHESTER D. ROCKWOOD.  
KENNETH L. OSMUN.